

# UNITED STATES PATENT OFFICE.

FRIEDRICH ALBERT KAUFMANN, OF PERTH AMBOY, NEW JERSEY, ASSIGNOR TO THE ROESSLER & HASSLACHER CHEMICAL CO., OF NEW YORK, N. Y., A CORPORATION OF NEW YORK.

## CEMENTATION PROCESS.

1,235,901.

Specification of Letters Patent. Patented Aug. 7, 1917.

No Drawing.

Application filed August 11, 1915. Serial No. 44,951.

To all whom it may concern:

Be it known that I, FRIEDRICH ALBERT KAUFMANN, a subject of the German Emperor, residing at the city of Perth Amboy, 5 in the county of Middlesex and State of New Jersey, have invented certain new and useful Improvements in Cementation Processes, of which the following is a specification.

10 The invention relates to the cementation of iron, steel and ferrous alloys and has for its object to provide an improved process to render the operation more efficient and economical than heretofore.

15 The improvement achieved by my invention consists essentially in employing hydrocyanic acid, in gaseous form, as "cementing agent" for iron, steel and other ferrous alloys. Hydrocyanic acid is easily obtainable 20 and has most perfectly the qualities necessary for cementation of steel; it is in gaseous condition at 26° C. and can be generated with the greatest ease from sodium cyanid, potassium cyanid and similar cyanid salts 25 by sulfuric acid or any other mineral or organic acid of sufficient strength to generate said gas from such cyanid salts. At an elevated temperature this gas decomposes into its constituents, of which the carbon is of

30 especial interest for the purposes of case-hardening or cementation, while the other constituents form ammonia which, as is well known, has a beneficial influence for the purpose in question. The carbon as formed 35

by the decomposition of hydrocyanic acid, or by decomposition of other gaseous cyanogen compounds diffuses in the presence of inert gases formed in the course of the process of decomposition or purposely added, 40 more freely and easily into the iron, steel and other ferrous alloys at a certain temperature, because it is then in *status nascendi*, and is therefore more effective than when under other conditions.

45 Owing to its catalytic properties, the presence of iron accelerates the decomposition of the gaseous cyanogen compounds.

The effect of the carbon derived from the decomposition of hydrocyanic acid or other 50 gaseous cyanogen compounds is more pronounced and more satisfactory and quicker than the effect obtained with other gaseous cementing agents, for instance, hydrocarbons, which as is well known, form "sudden" 55 cases, and which even after a long period

of treatment do not increase the depth of penetration of carbon in steel after reaching a certain depth. The treatment of steel at certain high temperatures by hydrocyanic acid or other gaseous cyanogen compounds 60 gives an excellent gradual case, *i. e.*, a gradual decrease of carbon content toward the heart of the piece; it also permits the regulation of the "penetration" with precision and certainty by regulating the amount of 65 gas applied and the length of time the material is subjected to the treatment.

The process consists essentially in the generation of hydrocyanic acid from cyanid salts by means of an acid, of which sulfuric 70 acid is perhaps the most economical when used in a suitable apparatus; I consider however, that the application of hydrocyanic acid derived by the reaction of cyanid salts with chemical compounds other than 75 acids, is also within the scope of my invention. The hydrocyanic acid so generated is introduced by suitable devices, either alone or diluted by a suitable inert gas purposely added into a furnace containing the steel or 80 other articles to be hardened, the furnace being heated to a temperature above approximately 700° C. The amount of gas and the length of time necessary for the process depends on the quality of hardening 85 effect desired. The time may vary from a few minutes to several hours according to the penetration of carbon to be obtained and the size of the steel or other articles to be hardened. At and above the aforesaid 90 temperature the gas will quickly decompose and the carbon so formed being in *status nascendi* and in the presence of inert gases, which inert gases may be decomposition products of the cyanogen compounds or may 95 be purposely added, or both, will easily penetrate the iron, steel or ferrous alloys to the desired depth and in the desired percentage. After thus being hardened by my new process the further treatment of the 100 steel or other material can be carried on by the ways well known to those skilled in the art.

I claim:

1. The process of cementing articles of 105 iron, steel or ferrous alloys, consisting in treating said articles with gaseous hydrocyanic acid at an elevated temperature.

2. The process of cementing articles of 110 iron, steel or ferrous alloys, consisting in

treating said articles with gaseous hydrocyanic acid at an elevated temperature in the presence of inert gaseous matter.

3. The process of cementing articles of iron, steel or ferrous alloys, consisting in treating said articles at approximately 700° C. with gaseous hydrocyanic acid.

4. The process of cementing articles of iron, steel or ferrous alloys, consisting in decomposing gaseous hydrocyanic acid at approximately 700° C. into carbon and ammonia and acting with the nascent carbon on the articles.

5. The process of cementing articles of iron, steel or ferrous alloys, consisting in decomposing gaseous hydrocyanic acid at approximately 700° C. into carbon and am-

monia and acting with the nascent carbon on the articles in the presence of the ammonia generated by the process.

6. The process of cementing articles of iron, steel or ferrous alloys, consisting in decomposing gaseous hydrocyanic acid at approximately 700° C. into carbon and ammonia and acting with the nascent carbon on the articles in the presence of the generated ammonia and other inert gases.

In testimony whereof I have signed this specification in the presence of two subscribing witnesses.

FRIEDRICH ALBERT KAUFMANN.

Witnesses:

CATHERINE A. COSTELLO,  
OTTO K. ZWINZENBERGER.